

P. BARTHEL.

## Treating Asphalt.

No. 135,879.

Patented Feb. 18, 1873.



Witnesses.

Chesler Thornton  
Henry Moore

### *Inventor*

Peter Barthel  
for Henry C. Roeder  
his attorney

# UNITED STATES PATENT OFFICE.

PETER BARTHEL, OF FRANKFORT-ON-THE-MAIN, GERMANY.

## IMPROVEMENT IN TREATING ASPHALT.

Specification forming part of Letters Patent No. 135,879, dated February 18, 1873.

*To all whom it may concern:*

Be it known that I, PETER BARTHEL, of the city of Frankfort-on-the-Main, in the Empire of Germany, have invented certain Improvements in Manufacturing Asphalt for Pavements and in the Apparatus employed in this process, of which the following is a specification:

The nature of my invention consists in the production of an asphaltic compound for pavements, which shall contain the durability and solidity of natural asphalts. To obtain this result I purify the natural asphalt from its mineral matters by the addition of sulphuret of carbon, or of benzine, and take from nine to twelve parts by weight of this purified asphalt, and then add from eighty-five to ninety parts by weight of powdered calcareous spar or marble, when the compound will be ready for use without any other addition.

The calcareous spar or marble to be used is first ground, and must then be sieved or washed to clean it of all dust, leaving only a fine sand, with particles of about equal size.

The asphalt is purified by means of an apparatus represented in the accompanying drawing.

A kettle, A, is arranged, having double walls, so that steam, produced in a boiler, R, can be introduced into the annular space between the two walls for the purpose of heating and dissolving the asphalt and other ingredients placed into the same. This kettle is partly filled with the asphalt to be purified together with sulphuret of carbon or benzine. Above the asphalt a sieve, L, made of silk or wire-gauze, is arranged, through which the dissolved materials have to pass, causing thereby the mineral impurities to fall back into the kettle. The solution passes then through a pipe, D, into a boiler, E, where the same is evaporated. The asphalt will remain in the boiler E, while the vapors of the sulphuret of carbon or of the benzine pass into the worm U, where the same are condensed, and the liquid

returned, through the pipe S, into the kettle A, to assist again in dissolving another quantity of asphalt. The pipe S enters the inner part of the kettle A near its bottom. The boiler E is inclosed in a casing or jacket, into which steam is admitted, through the pipe H, from the steam-boiler R, whereby the dissolving liquids, such as sulphuret of carbon or benzine, are evaporated. At the same time an ordinary furnace, F, is arranged under this boiler E, so that those particles of the dissolving liquids which cannot be evaporated at the temperature of the steam can be evaporated by the direct heat of the furnace.

When the asphalt is dissolved by means of sulphuret of carbon some heavy mineral oil must be added to the asphalt, so that the required elasticity may be obtained. The quantity of mineral oil necessary varies from two to five per cent., according to the nature and quality of the natural asphalt, and may be put either into the kettle A or into the boiler E.

When benzine is used as the dissolving agent this addition of mineral oil is not required, as enough of the heavier parts of the benzine remains in the asphalt to obtain the desired elasticity.

What I claim as my invention, and desire to secure by Letters Patent, is—

1. The arrangement of a sieve, L, in the kettle A above the material to be dissolved, substantially as and for the purpose hereinbefore set forth.

2. The combination of the kettle A, boiler E, and worm U, connected together in the manner and for the purpose substantially as set forth.

3. The combination of asphalt, purified of its mineral impurities, with the sand of calcareous spar or marble in the proportions and for the purpose substantially as described.

PETER BARTHEL.

Witnesses

FERDINAND CAPITAINE,  
WILH. SARTORIUS.